

## 1

3,031,254

**PROCESS OF DELUSTERING ACETONE-SOLUBLE CELLULOSE ACETATE TEXTILE WITH A HOT SOAP SOLUTION CONTAINING HYDROGEN PEROXIDE**

Dennis Grady, Harold Bates, and James Wotherspoon Fisher, Spondon, near Derby, England, assignors to British Celanese Limited, a corporation of Great Britain No Drawing. Filed Sept. 9, 1955, Ser. No. 533,506 Claims priority, application Great Britain Oct. 1, 1954 3 Claims. (Cl. 8—131)

This invention relates to the treatment of textile and other materials of cellulose acetate for the purpose of effecting a reduction in their lustre.

It is well known that the lustre of bright textile materials of acetone-soluble cellulose acetate can be reduced by subjecting the material to a suitable hot aqueous treatment. For this purpose treatment with an aqueous soap solution at or near the boil is largely employed commercially. The ease with which loss of lustre takes place varies somewhat according to the particular acetone-soluble cellulose acetate of the material. Some materials lose lustre relatively easily and can be given a more or less completely mat appearance by a treatment for 1½ hours in a 5 gram per litre soap solution at 99° C. Others are somewhat less delustered by such a treatment but have the advantage that when a bright finish is required they can readily be dyed in the soap baths conventionally used for dyeing cellulose acetate at temperatures up to perhaps 85° C. with little risk of loss of lustre.

Various substances have been proposed for addition to the aqueous soap baths in order to accelerate the delustering action of the latter or to permit a greater reduction of lustre. Examples of such substances are phenol, pine oil, methylcyclohexanol, terpineol and naphthalene but none are entirely satisfactory. Some are not effective to a worthwhile extent, some add unreasonably to the cost of the process, some result in a very considerable loss in the strength of the material while some, for example phenol and naphthalene, are difficult to remove to the extent necessary if the material is not to have an unwanted odour.

We have now found that hydrogen peroxide can be used to increase the delustering action of hot aqueous delustering liquids on textile and other material of acetone-soluble cellulose acetate. The material may be subjected to the action of the hydrogen peroxide before the termination of delustering by the liquid. Thus we have found that material which has been treated with aqueous hydrogen peroxide, for example hydrogen peroxide in aqueous soap solution at 65° C., loses lustre more rapidly than the untreated material when it is subjected to an aqueous soap solution at or near the boil. We have obtained the best results however by simply including hydrogen peroxide in the hot aqueous delustering bath itself. Thus by treatment at or near the boil (97 to 100° C.), e.g. at 99° C., for 1½ hours in a 5 grams per litre soap solution to which has been added 1 cc. per litre of hydrogen peroxide (130 volumes) a full deluster can be obtained on a bright cellulose acetate yarn or fabric, e.g. a satin fabric, which is only partially delustered by a similar treatment omitting the hydrogen peroxide.

The use of hydrogen peroxide in this way results in a product of acceptable strength and does not impart unwanted odour. Further, the material is simultaneously bleached so that a separate bleaching operation is unnecessary.

The preferred delustering bath is an aqueous soap solution containing about 5 grams of soap per litre. Hydrogen peroxide is however an effective delustering accelerator for lower or higher concentrations of soap, e.g. con-

## 2

centrations down to 1 or 2 grams per litre or up to 8 or 10 grams per litre.

The concentration of hydrogen peroxide in the soap solution may vary within quite wide limits. Excellent results can be obtained by using from 1 to 5 ccs. per liter of hydrogen peroxide (130 volumes). Lower concentrations can be used, for example 0.75 cc. per litre and satisfactory results obtained, but concentrations as low as 0.5 cc. per litre generally lead to decidedly inferior results.

The hydrogen ion concentration of the delustering bath is of some importance for best results. We find that the delustering effect increases as the pH value of the bath increases from about 7.0 to about 9.5 but at higher pH value tends to fall off somewhat. It is preferred to effect the delustering treatment at a pH value of 8.5 to 9.

In the case of treating cellulose acetate fabric it is preferred to apply the treatment to material which is substantially free from size. A soap delustering bath may then be used a number of times if hydrogen peroxide is added, after each batch of material has been treated, to bring the concentration of hydrogen peroxide back to the desired level. The hydrogen peroxide initially present is by no means all decomposed during a delustering treatment of 1½ hours at 99° C. If desired, however, the treatment may be applied to cellulose acetate fabrics carrying the weaving size, the treatment then serving both to remove size from the material and to effect delustering. In this case it is preferred to use a fresh soap bath for each batch of material since otherwise size and other products accumulate in the bath and appear to diminish the delustering action. If desired, after delustering the material in the manner described, it may be given a scouring treatment, for example with an alkali metal salt of a long chain alkyl sulphate type of detergent, for the purpose of removing any unwanted fatty acid or difficultly soluble metallic soap from the material.

While the process can be used for the treatment of cellulose acetate yarns it is of most value for the treatment of fabrics. The latter may be subjected to the action of the delustering bath in any convenient way, for example by suspending them in the form of hanks of fabric in the delustering liquor.

It is surprising that the hydrogen peroxide is so effective in accelerating the delustering action of the hot aqueous liquids on acetone-soluble cellulose acetate since we find that other oxidising bleaching agents seem to have little effect or very much less effect on the rate of delustering. This applies for instance to sodium percarbonate and to sodium hypochlorite.

We do not exclude the use of hydrogen peroxide produced in the delustering bath by suitable means.

Aqueous solutions of detergent cationic or anionic surface-active agents other than sodium or other alkali metal soaps of fatty acids may likewise have their delustering action increased by means of hydrogen peroxide. Such surface-active agents may be quaternary ammonium compounds (in the form of water-soluble salts) containing an un-substituted alkyl group having a chain of at least 10 successive carbon atoms united by carbon to carbon linkages, for example cetyl-trimethyl-ammonium chloride or bromide. Again they may be acid sulphates or acid phosphates (in the form of water-soluble salts) of monohydroxylated aliphatic hydrocarbons having a chain of at least 10 successive carbon atoms united by carbon to carbon linkages counting from and including the carbon atom carrying the hydroxyl group, for example lauryl sulphate, palmityl sulphate, stearyl sulphate, or oleyl sulphate, or the sulphate of a mixture of such alcohols as can be obtained by reduction of the esters of the mixture of fatty acids found in cocoanut

oil. Detergent of the alkylarylsulphonate type may likewise be employed. Such surface-active agents are, however, generally inferior to soaps as delustring agents for cellulose acetate and when used in the presence of hydrogen peroxide are likewise inferior to aqueous solutions of soap used in the presence of hydrogen peroxide.

The invention is illustrated by the following example:

*Example*

A loom state satin fabric consisting entirely of yarns of acetone-soluble cellulose acetate of a kind which cannot be completely delusted by treatment for 1½ hours in a 5 grams per litre soap solution at 99° C., is desized by a treatment for ½ hour at 85° C. in a 5 grams per litre solution of soap-flakes in water. The de-sized material, in the form of a hank, is then immersed in an aqueous bath containing 5 grams per litre of soap-flakes and 1 cc. per litre of hydrogen peroxide (130 volumes). The temperature of the bath is then raised to 99° C. and is maintained at this for 1½ hours, the hank of fabric being turned at intervals to ensure even treatment. The material is then lifted from the delustring bath and scoured at 65° C. for 30 minutes in an aqueous bath containing per liter 2 cc. of ammonia and 0.2 gram of Pentrone T, a fatty alcohol sulphate. This operation may be carried out on a winch. Finally the material is washed off, hydro-extracted and dried on a pin stenter.

The fabric is thus given a dull finish which is much duller than is obtained if the delustring operation is effected with aqueous soap solution only without the addition of hydrogen peroxide.

Though the invention is primarily of value in the delustring of textile material of acetone-soluble cellulose acetate, it may be used in connection with the delustring of textile material of other types of cellulose acetate

which are susceptible to reduction of lustre by hot aqueous treatments, for example to textile materials of this kind of which the cellulose acetates are of acetyl values ranging up to that of a cellulose triacetate. The new process may also be applied for the delustring of cellulose acetate in other forms, for example foils or films of acetone soluble cellulose acetate.

Having described our invention what we desire to secure by Letters Patent is:

- 10 1. In a process wherein textile material of acetone-soluble cellulose acetate is delusted by the action of a hot aqueous solution of soap the solution having a pH value of 7 to 9.5, increasing the delustring action of the solution by including hydrogen peroxide therein in an amount per litre equivalent to from 1 to 5 ccs. of hydrogen peroxide of 130 volume strength.
- 15 2. Process according to claim 1 in which said hot aqueous solution of soap has 1 to 10 grams of soap per litre and is at a temperature of 97 to 100° C.
- 20 3. Process according to claim 1 in which said hot aqueous solution of soap has about 5 grams of soap per litre, a pH of 8.5 to 9 and a temperature of 97 to 100° C. in which said treatment has a duration of about 1½ hours and in which said solution contains per litre hydrogen peroxide equivalent to about 1 cc. of hydrogen peroxide of 130 volume strength.
- 25

References Cited in the file of this patent

UNITED STATES PATENTS

2,264,415 Taylor ----- Dec. 2, 1941

FOREIGN PATENTS

388,520 Great Britain ----- Mar. 2, 1933

394,333 Great Britain ----- June 21, 1938